

Jan. 8, 1929.

1,697,858

A. FIEDLER

LUBRICATED MOTION PICTURE FILM AND METHOD OF MAKING THE SAME

Filed May 26, 1924



INVENTOR  
*Albert Fiedler*  
BY  
*Charles Holland*  
ATTORNEY

## UNITED STATES PATENT OFFICE.

ALBERT FIEDLER, OF WEEHAWKEN, NEW JERSEY.

## LUBRICATED MOTION-PICTURE FILM AND METHOD OF MAKING THE SAME.

Application filed May 26, 1924. Serial No. 715,948.

My invention relates to motion picture films having a lubricant along the perforated edges thereof to enable them to move easily through the projecting machine. More particularly my invention contemplates a motion picture film of the kind described in which the applied lubricant will cohere with and on drying become incorporated in the gelatine surface of the film so that it will be incapable of being rubbed off by objects with which it comes into contact.

It has been the experience of the motion picture industry that prints of motion pictures made at a considerable cost upon celluloid strips are frequently torn while they are being run through the projecting machine in the theatres or exhibition houses. This tearing ordinarily occurs at the edge of the celluloid print which contains a series of perforations designed to accommodate the cogs of the sprocket wheel that moves the film through the machine. The film, when it is placed in the projecting machine, is drawn through it at a considerable speed. The projecting machine is provided with an opening in the machine head in front of a strong light. The film as it is drawn through the machine must pass down before this opening in order that the light behind it may project the picture on to the screen. A hinged "gate" provided with an opening corresponding to that in the machine head, closes against the film in order to compel it to move evenly before the light. The interval between the gate and the machine head is hardly greater at the perforated edges than the thickness of the film and the film is in constant contact with both as it moves through. The portions of the gate and of the machine head that come in contact with the celluloid film tend to become extremely hot and remnants of gelatine from the face of the films adhere to the gate or to the machine head and are baked hard and frequently carbonized. After a period of time it frequently happens that an accumulation of this hard rough material forms in the narrow passage between the gate and machine head and has a tendency to hold back the film in its progress and to catch in perforations at the edge with result that the perforated edge of the film becomes torn.

It is the object of the present invention to provide a motion picture film to the perforated edges of which a lubricant has been ap-

plied at the time the print is completed in the laboratory and before it is released for exhibition purposes. It is a further object of the invention to provide a process for applying this coating of lubricant to the said perforated edges of the film. To this end, I prefer to use a compound of which the base is a gelatinous material and an oil, preferably gelatine and cocoanut oil, as described in my co-pending application, Serial Number 41,202, filed July 2nd, 1925, which forms a division of this application. When the mixture is thoroughly stirred the compound is ready to be applied to the film. Other gelatinous materials, however, may be used with very favorable results. Among these materials I may mention agar-agar and plastic materials such as celluloid, gum arabic, shellac and the like. Similarly instead of cocoanut oil, I may use with good effect a number of other vegetable or animal oils. Alcohol may be replaced by any easily volatilized material.

This application may be made in any known manner, as for instance, by causing the edges of the film to run through a bath of the compound while it is still hot. The material coheres with the gelatine surface of the film and becomes apparently a part thereof but does not affect the unsurfaced celluloid at the back of the film. When the film is withdrawn from the bath the composition cools and the alcohol contained in it causes speedy drying by its evaporation and the edges of the film are then well lubricated and so dry that the compound will not rub on to the hands or upon the objects with which it comes in contact.

It is nevertheless very slippery and enables the film to slide smoothly through the narrow passage between the gate and the head of the projecting machine.

It frequently happens that in removing the film from the bath the lubricant fills the perforations of the film and if allowed to dry would impair the movement of the film through the projecting machine. This, however, can easily be avoided by passing the perforated edges through a jet of air while the lubricant is still in a moist condition so that the perforations are blown clear of this surplus material.

Furthermore, it is not necessary to apply the composition to the film while hot as it may be desirable to apply the liquid cool or

in a slightly warm state to the film at the time the photographically sensitive gelatine coating is placed upon the base thereof in which case it will set together with the gelatine coating. It may also be applied in a cool state to the finished film, when, for example, before the film is printed, the application of heat might be injurious.

The drawing shows a portion of a film 10 which has been lubricated according to my invention; the legends upon which designate the various parts.

What I claim and desire to secure by Letters Patent:

15 1. A motion picture film comprising a celluloid strip, a sensitive photographic coating on one side thereof, except at the edges, and a coating of a lubricating material consisting of gelatin and oil dissolved in water and alcohol on both edges of the sensitive side.

20 2. A motion picture film comprising a photographically non sensitive base, a photographically non sensitive lubricant consisting of gelatin and oil dissolved in water and alcohol 25 coated directly on the edges of said base and a photographically sensitive coating on one side between said coatings of lubricant.

25 3. The process of lubricating motion picture films by heating a compound of gelatine and oil dissolved in water and alcohol; then when the temperature of the solution is sufficiently high to soften the gelatine surface of the film, applying the compound to the edges 30 thereof and allowing it to dry thereon; where-

by the compound is incorporated into the gelatine surface of the film.

4. The process of lubricating motion picture films by applying a compound consisting of gelatine and oil dissolved in water and alcohol to the edges of the film. 40

5. A motion picture film comprising a celluloid strip, one side of which bears a central path having a sensitive photographic coating and paths at the edges of said sensitive path 45 coated with lubricating material consisting of gelatin and oil dissolved in water and alcohol.

6. A motion picture film comprising a base of photographically non sensitive material, 50 coatings of lubricating material consisting of gelatin and oil dissolved in water and alcohol affixed to said base at the edges and on one side a coating photographically printed between said coatings of lubricating material. 55

7. A motion picture film having coatings of lubricating material consisting of gelatin and oil dissolved in water and alcohol on both edges and on one side a coating of photographically sensitive material between said 60 coatings of lubricating material.

8. A motion picture film having coatings of lubricating material consisting of gelatin and oil dissolved in water and alcohol on both edges and on one side a coating of material 65 bearing a photographic print between said coatings of lubricating material.

In witness whereof, I have subscribed my name hereto this 15th day of May, 1924.

ALBERT FIEDLER.